

Patented Nov. 6, 1928.

1,690,427

# UNITED STATES PATENT OFFICE.

NORMAN E. OLIVER, OF NEW YORK, N. Y., ASSIGNOR TO HERMETITE CORPORATION, OF NEW YORK, N. Y., A CORPORATION OF NEW JERSEY.

## PROCESS FOR THE COATING OF PERVERSUS MATERIAL.

No Drawing.

Application filed May 29, 1925. Serial No. 33,636.

My invention relates to processes for the treatment of fabrics and other pervious materials and refers particularly to the treatment of such materials with the retention of softness and pliability.

It is frequently desirable to cover, or coat, pervious materials, as, for instance woven fabrics, with a surface material for purposes of rendering them water proof or fire proof or for decorative or other purposes.

The coating materials employed for this purpose may be lacquers, varnishes, cellulose or celluloid compounds and mixtures which impart valuable properties to the materials thus treated.

The employment of these, and similar, coating materials has been considerably limited because of the harshness of the treated results. Attempts have been made to overcome this objectionable quality by incorporating softening materials with the coating compounds or employing them in the coating process.

Among the softening agents thus employed are vegetable oils, such as castor oil, their sulphurated products and other oils and greases. Many of these oils are objectionable because of their rancidity, liability to injure the fiber and tendency to break down the coating compound with the formation of objectionable products.

I have found that there are two general reasons for the reduction of the pliability of materials of the character described when they are coated, or covered, with the mentioned and similar coating compounds.

The one reason is the stiffness and non-pliability of the coating compound itself, which permeates the fabric, whether the material be passed through a solution of the coating compound or the solution be applied to the ordinary woven or pervious material. This positioning of the coating compound within the fabric and between and around the fibers results in material having the physical properties of the coating compound to a large degree. This decreased pliability of the fabric is still further enhanced by the fact that the coating compounds are usually of such a nature as to adhere to the fibers, thus producing a practically solid mass of the coating compound with the fibers enclosed therein.

The other general reason for the production of coated goods of less pliability than the original material is based upon the fact that in many coating operations, and especially

in those methods in which the fabric is immersed in a solution of the coating compound, a proportion of the contained fiber oils, fats and softening agents is removed and in these cases the original pliability can not be regained by attempted replacement of the removed products.

It is evident, therefore, that the logical method for coating fabrics and other pervious materials is the retention of the original oils, the non-saturation of the material with the coating compound and the employment of a pliable coating compound.

The process of my invention possesses all of the last described desirable attributes, overcomes all of the objectionable features incident to previously known methods, and produces a coated material possessing softness and pliability.

All pervious materials have a plurality of openings therethrough, those in woven fabrics being the spaces between the several fibers. These openings have capillary attraction, the degree of capillarity being dependent upon the size of the openings, and it is through the medium of this capillary attraction that the solution of coating compounds is drawn, or carried, into the interior of the fabric.

I overcome this objectionable feature by treating the material previous to coating in such a manner and by such means that the elements making up the material, as for instance the fibers in woven fabrics, will swell, thus reducing the size of the openings, or interstices, therein, and the same result can be accomplished if the treating material is of such a character that it will fill up and hence close the openings, preventing a subsequently applied coating material from entering therein. Further, the treating material may be of such a character as to produce both of the foregoing described results. For purposes of simplicity of description, I refer to the foregoing treating materials in my specification and claims as "treating materials".

The following is one example of the process of my invention:—

I coat one side of a fabric with a treating material, as glucose, and then coat the other side of the fabric with a solution of a pliable coating material, as a solution containing 100 parts nitrocellulose to over 60 parts of tricresylphosphate, and dry. I then wash the fabric in a solution of soap and water, or in a

solution of oil emulsified in water, to remove the glucose, and dry.

The treating material, as glucose or the like, is applied to one side of the fabric as a film 5 coating, and operates to prevent the solution of the coating material, which forms the pliable coating at the other side, from going through.

I prefer to employ treating materials which 10 are soluble in water or which can be removed by some other solvent.

If desirable, I can apply steam, or moisture, to the uncoated side of the material in order 15 to reproduce the original woven appearance upon the coated side.

By "after-treating" the material as used in my specification and claims, I mean treating the coated material with a solvent of the 20 treating material, with or without an oil or softening material, or with steam or moisture.

By "coating compounds" and "coating materials" in my specification and claims, I mean those products, either singly or in combination which can be applied to pervious 25 materials and which become affixed thereto by the steps of my process.

I do not limit myself to the particular materials, quantities, temperatures or steps 30 of process particularly described, as these are given in order to clearly explain the process of my invention.

Reference may also be had to my co-pending application for patent, Serial No. 33,635, filed in conjunction with the present case, 35 and in which a similar process for effecting the results herein obtained is set forth.

What I claim is:

1. In a process for coating a pliable pervious material, first subjecting only one side 40 of said material to a treating step which closes or reduces the size of the interstices or pores thereof, and then applying to the other side of said treated material a coating material of the class comprising cellulose, celluloid compounds or mixtures, lacquers, varnishes or the like, which will remain pliable in the coating and produce at said coated side a finished surface retaining the pliability and appearance 45 of the pervious material.

2. In a process for coating a pliable pervious material, first subjecting only one side of said material to a treating step which closes or reduces the size of the interstices or 55 pores thereof, then applying to the other side of said treated material a coating material of the class comprising cellulose, celluloid compounds or mixtures, lacquers, varnishes or the like, which will remain pliable in the coating and produce at said coated side a finished surface retaining the pliability and appearance 60 of the pervious material, and then drying the coated side of said treated material.

3. In a process for coating a pliable pervious material, first subjecting only one side 65

of said material to a treating step which closes or reduces the size of the interstices or pores thereof, then applying to the other side of said treated material a coating solution which will remain pliable in the coating and 70 which contains approximately 100 parts of nitrocellulose to over 60 parts of tricresylphosphate, and then drying said coating solution to produce at said coated side a finished surface retaining the pliability and appearance 75 of the pervious material.

4. In a process for coating a pliable pervious material, subjecting one side of said material to a treating step which closes or reduces the size of the interstices or pores thereof, treating the other side of said pervious material with a coating material of the class comprising cellulose, celluloid compounds or mixtures, lacquers, varnishes or the like, which will remain pliable in the coating and produce at said coated side a finished surface 80 retaining the pliability and appearance of the pervious material, drying said pliable coating material, after-treating the treated material by the application of steam or moisture, and again drying the treated material.

5. In a process for coating a pliable pervious material, applying glucose to one side of said material, treating the other side of said material with a coating material of the class comprising cellulose, celluloid compounds or mixtures, lacquers, varnishes or the like, which will remain pliable in the coating and produce at said coated side a finished surface 85 retaining the pliability and appearance of the pervious material, drying said pliable coating material, after-treating the treated material by the application of steam or moisture, and again drying the treated material.

6. In a process for coating a pliable pervious material, subjecting one side of the material to a filling material of the class comprising glucose, or the like, which will close or reduce the size of the interstices or pores 90 of the pervious material, treating the other side of said material with a coating solution which will remain pliable in the coating and which contains approximately 100 parts of nitrocellulose to over 60 parts of tricresylphosphate, drying said coating solution, 95 after-treating the treated material to remove the first-mentioned filling material, and again drying the treated material.

7. In a process for coating a pliable pervious material, first subjecting one side of said material to a filling material of the class comprising glucose, or the like, which will close or reduce the size of the interstices or pores 100 of the pervious material, then applying to the other side of said treated material a coating material of the class comprising cellulose, celluloid compounds or mixtures, lacquers, varnishes or the like, which will remain pliable in the coating and produce at 105 said coated side a finished surface retaining the pliability and appearance of the pervious material.

the pliability and appearance of the pervious material, and then removing the first-mentioned filling material.

8. In a process for coating a pliable pervious material, first subjecting one side of said material to a filling material of the class comprising glucose, or the like, which will close or reduce the size of the interstices or pores of the pervious material, then applying to the other side of said treated material a coating material of the class comprising cellulose, celluloid compounds or mixtures, lacquers, varnishes or the like, which will remain pliable in the coating and produce at said coated side a finished surface retaining the pliability and appearance of the pervious material, drying said pliable coating, then removing the first-mentioned filling material, and again drying the treated material.

9. In a process for coating a pliable pervious material, first subjecting one side of said material to a filling material of the class comprising glucose, or the like, which is soluble and will close or reduce the size of the interstices or pores of the pervious material, then applying to the other side of said treated material a coating material of the class comprising cellulose, celluloid compounds or mixtures, lacquers, varnishes or the like, which will remain pliable in the coating and produce at said coated side a finished surface retaining the pliability and appearance of the pervious material, drying said pliable coating, and then subjecting the treated material to the action of a material for reproducing at that side the original appearance of the pervious material.

10. In a process for coating a pliable pervious material, first subjecting one side of said material to a filling material of the class comprising glucose, or the like, which is soluble and will close or reduce the size of the interstices or pores of the pervious material, then applying to the other side of said treated material a coating material of the class comprising cellulose, celluloid compounds or mixtures, lacquers, varnishes or the like,

which will remain pliable in the coating and produce at said coated side a finished surface retaining the pliability and appearance of the pervious material, drying said pliable coating, then subjecting the treated material to the action of a solvent of the first-mentioned filling material, and again drying the treated material.

11. In a process for coating a pliable pervious material, first subjecting one side of said material to a filling material of the class comprising glucose, or the like, which will close or reduce the size of the interstices or pores of the pervious material, then applying to the other side of said treated material a coating material of the class comprising cellulose, celluloid compounds or mixtures, lacquers, varnishes or the like, which will remain pliable in the coating and produce at said coated side a finished surface retaining the pliability and appearance of the pervious material, drying said pliable coating, and then subjecting the uncoated side of the treated material to the action of a material for reproducing at that side the original appearance of the pervious material.

12. In a process for coating a pliable pervious material, first subjecting one side of said material to a filling material of the class comprising glucose, or the like, which is soluble and will close or reduce the size of the interstices or pores of the pervious material, then applying to the other side of said treated material a coating material of the class comprising cellulose, celluloid compounds or mixtures, lacquers, varnishes or the like, which will remain pliable in the coating and produce at said coated side a finished surface retaining the pliability and appearance of the pervious material, drying said pliable coating, and then subjecting the treated and coated material to the action of a solvent of the first-mentioned filling material.

In testimony whereof I have signed this 90 specification.

NORMAN E. OLIVER.